

## 1

3,029,204

ACIDIC PARTIAL ESTERS AS LUBRICATING  
OIL ADDITIVES

Alfred H. Matuszak, Westfield, and Stephen J. Metro, Scotch Plains, N.J., and John Samuel Paul Schwarz, Dugway Proving Ground, Utah, assignors to Esso Research and Engineering Company, a corporation of Delaware

No Drawing. Filed May 12, 1959, Ser. No. 812,583  
9 Claims. (Cl. 252—56)

This invention relates to lubricating oil additives for improving the load-carrying ability of a lubricant and for inhibiting corrosion of lead. Particularly, the invention relates to synthetic ester lubricating oil compositions containing acidic partial esters which are prepared by esterification reactions between dicarboxylic acids and glycols.

The use of various fully esterified aliphatic diesters and complex esters as synthetic lubricating oils is well known to the art and has been described in numerous patents, e.g. U.S. 2,723,286; 2,743,234; and 2,575,196. In general, these prior aliphatic synthetic ester lubricating oils are characterized by viscosity properties that are outstanding at both low and high temperatures, especially when compared to mineral lubricating oil. Because of these characteristics, the synthetic ester oils have become of increasing importance in the field of lubrication. And one of the most important current applications of such compounds is in the lubrication of aviation gas-turbine systems such as are used in the "turbo-jet" or "turbo-prop" type of aircraft. However, in general, the load-carrying ability of the aliphatic ester oils is not particularly high. Because of the increasing severity of the conditions prevailing in the lubrication of aviation gas-turbine systems it is highly desirable to form synthetic ester lubricating compositions which have higher load-carrying ability than is now generally available. At the same time the composition should be noncorrosive to lead in the copper-lead bearings generally present in aircraft engines. It has now been found that the acidic partial esters of this invention are very effective in synthetic ester lubricating oil compositions not only for improving load-carrying ability but also for inhibiting lead corrosion by the ester oil. At the same time, these new additive materials do not unduly attack copper, magnesium, aluminum or silver which are generally also present in the engine.

The acidic partial esters of the invention are believed to be represented by the following formula:

Dibasic Acid-Glycol-(Dibasic Acid-Glycol)<sub>x</sub>-Dibasic Acid wherein  $x$  is a number of 0 to 4. This acidic material is prepared by simple esterification reactions between a glycol and a dicarboxylic acid using about 1.2 to 2.0, preferably 1.7 to 2.0 moles of the dicarboxylic acid per mole of the glycol. When using two moles of acid per mole of glycol, the primary product is believed to have the formula: Dibasic Acid-Glycol-Dibasic Acid, i.e.  $x$  is 0. However, minor amounts of longer chain molecules are undoubtedly also present, i.e. where  $x$  is 1 or more, and the exact composition is not known with certainty.

The dicarboxylic acids used in preparing the acidic partial ester will include the  $C_6$  to  $C_{12}$  alkandioic acids, such as adipic, sebacic, azelaic and isosebacic acid. The isosebacic acid is a mixture of  $C_{10}$  acids comprising about 60 to 90 weight percent of  $\alpha$ -ethyl suberic acid, about 5 to 25 weight percent of  $\alpha, \alpha'$ -diethyl adipic acid, and about 5 to 15 weight percent of sebacic acid. A typical acid will contain about 75 weight percent of  $\alpha$ -ethyl suberic acid, about 15 weight percent of  $\alpha, \alpha'$ -diethyl adipic acid and about 10 weight percent of sebacic acid.

The glycol, which is used, may be either an alkylene

## 2

glycol or a polyalkylene glycol, said glycol containing a total of 2 to 36, preferably 4 to 18, carbon atoms. Thus, included in the invention are ethylene glycol, propylene glycol, butanediol-1,4, pentanediol-1,5; hexanediol-1,6, octylene glycol, and other straight or branched chain hydrocarbon glycols. Operable polyglycols will include polyethylene glycols of the formula



10 wherein  $n$  is 1 to 17, preferably 1 to 8, and polypropylene glycol of the formula



15 wherein either  $\text{R}_1$  or  $\text{R}_2$  is a methyl group and the other is hydrogen, and  $n$  is 1 to 11, preferably 2 to 5.

The esterification reaction is preferably carried out in the absence of an esterification catalyst. While the reaction will take place more rapidly with a catalyst, a catalyst is not used in order to obtain a purer reaction product and to avoid washing procedures to eliminate the catalyst. If desired a water entraining agent such as heptane or toluene may be used.

20 The ester oils operable as base oils in the compositions of this invention comprise hydrocarbon chains interrupted with ester linkages. The hydrocarbon chains may be further interrupted with ether or thioether linkages. Such esters will include diesters, polyesters, and complex esters.

25 The diesters are prepared from dicarboxylic acids fully esterified with monohydric alcohols, or from glycols fully esterified with monocarboxylic acids. The total number of carbon atoms in the diester molecule is about 20 to 36, preferably 22 to 26. Preferred dicarboxylic diesters are 30 those of the formula:



35 wherein each R may be the same or different and represents the straight or branched chain alkyl radical of an alkanol having about 6 to 13 carbon atoms, and  $\text{R}'$  is a straight or branched chain  $C_2$  to  $C_8$  divalent saturated aliphatic hydrocarbon radical. Examples of such diesters include: di-2-ethylhexyl sebacate, di-n-nonyl adipate, di- $C_8$  Oxo azelate, di-n-heptyl isosebacate, di- $C_{10}$  Oxo adipate, di- $C_8$  Oxo adipate, di-2-ethylhexyl adipate, di- $C_7$  Oxo adipate, di- $C_8$  Oxo trimethyl adipate, di- $C_{13}$  Oxo pimelate, etc. Other operable diesters are those prepared from glycols and monocarboxylic acids such as dipropylene glycol dipelargonate and polyethylene glycol 200 dicaprate.

40 Diesters prepared from the Oxo alcohols, which are isomeric mixtures of branched chain aliphatic primary alcohols, are particularly desirable. The Oxo alcohols have a very high degree of branching in the hydrocarbon chain, which results in diester oils having low pour points and low viscosity at low temperature. These alcohols are prepared from olefins, such as polymers and copolymers of  $C_3$  and  $C_4$  monoolefins, which are reacted with carbon monoxide and hydrogen in the presence of a cobalt-containing catalyst such as a cobalt carbonyl catalyst, at temperatures of about 300° to 400° F., and under pressures of about 1000 to 3000 p.s.i. to form aldehydes.

45 The resulting aldehyde product is then hydrogenated to form the Oxo alcohol which is then recovered from the hydrogenation product.

50 Operable polyesters are prepared by reacting polyhydric alcohols such as trimethylolpropane and pentaerythritol with monocarboxylic acids such as butyric acid, caproic acid, caprylic acid, pelargonic acid, etc. to give the corresponding tri- or tetraesters.

55 The complex esters which may be used as the base oils are formed by esterification reactions between a dicarboxylic acid, a glycol, and an alcohol and/or a mono-

carboxylic acid. These esters may be represented by the following formulas:



wherein  $R_1$  and  $R_5$  are alkyl radicals of a monohydric alcohol (e.g. alkanols), or a monocarboxylic acid (e.g. alkanoic acids),  $R_2$  and  $R_4$  are hydrocarbon radicals of dicarboxylic acids (e.g. alkandioic acids), and  $R_3$  and  $R_6$  are divalent hydrocarbon or hydrocarbon-oxy radicals, such as  $-\text{CH}_2(\text{CH}_2)_n-$  or



or  $-\text{CH}_2\text{CH}(\text{CH}_3)\text{OCH}_2\text{CH}(\text{CH}_3)-$ , derived from an alkylene glycol or polyalkylene glycol. "n" in the complex ester molecule, will usually range from 1 to 6 and is controlled by the relative molar ratio of the glycol or polyglycol to the dicarboxylic acid. In preparing the complex ester, there will always be some simple ester formed, i.e.  $n=0$ , but this will generally be a minor portion.

Some specific materials used in preparing the above types of complex esters are as follows: alkanols having 6 to 13 carbon atoms such as n-butyl alcohol, 2-ethylbutyl alcohol, 2-ethylhexanol, n-hexyl alcohol,  $C_8$  Oxo alcohol and  $C_{10}$  Oxo alcohol, etc.; the corresponding fatty or monocarboxylic acids; dicarboxylic acids and glycols of the same type described as useful in the preparation of the acidic partial esters of the invention. In addition the corresponding thioglycols may be used. In general these complex esters will have a total of 20 to 80, preferably 30 to 50, carbon atoms. These complex esters and methods for their preparation are known in the art and have been described in various patents.

The lubricating compositions of the invention will comprise a major proportion of a synthetic ester lubricating oil and about 0.01 to 2.0%, preferably 0.1 to 0.5 wt. percent of the acidic partial ester additive. The composition can also include other additives (e.g. 0.01 to 10.0 wt. percent) such as oxidation inhibitors such as phenothiazine, phenyl- $\alpha$ -naphthylamine, p-amino diphenyl amine; viscosity index improvers such as polymethacrylates, polystyrene; anti-foamants such as dimethylsilicone polymers; anti-wear agents; additional load-carrying agents; corrosion inhibitors; etc.

The invention will be further understood by the following examples:

#### EXAMPLE I

An acidic partial ester was prepared as follows:

Into a 1,000 ml. round-bottom 3-neck flask fitted with a stirrer, thermometer and a reflux condenser with a water trap was placed 808 grams (4.0 moles) of sebacic acid and 364 grams (2.0 moles) of Polyethylene Glycol 200 (PEG 200—a commercial polyglycol having an average molecular weight of about 182). 60 ml. of heptane as a water entraining agent was also introduced. No esterification catalyst was employed. The mixture was then refluxed at atmospheric pressure and to a final liquid temperature of 225° C. while stirring for 2 hours. The calculated amount of water (4 moles) was collected in the trap. The resulting residue was stripped of volatiles at 200° C. under a jet of nitrogen and about 1100 grams of a white semi-solid acidic partial ester was obtained. This material may be represented by the following word formula:

Sebacic acid-PEG 200-Sebacic acid

#### EXAMPLE II

2 moles of sebacic acid was reacted with 1 mole of hexanediol-2,5 following the procedure of Example I.

#### EXAMPLE III

4 moles of adipic acid was reacted with 2 moles of

Polyethylene glycol 200 following the procedure of Example I.

#### EXAMPLE IV

2 moles of adipic acid was reacted with 1 mole of hexanediol-2,5 following the procedure of Example I.

#### EXAMPLE V

2 moles of adipic acid was reacted with 1 mole of 2-ethyl-hexanediol-1,3 following the process of Example I.

The products of Examples I through V, described above, were added to a diester base oil composition and tested for lead corrosion. The diester base composition was a 50/50 volume mixture of a di- $C_8$  Oxo adipate and a di- $C_{10}$  Oxo adipate which mixture contained 1 wt. percent of phenothiazine as an oxidation inhibitor. The Oxo portions of the adipates were derived from Oxo alcohols prepared from a  $C_8$ - $C_4$  olefin feed.

Several of the products of Examples I through V were also added to a complex ester having the general formula:



wherein  $x$  averaged about 1.7. This complex ester also contained 0.5 wt. percent of phenothiazine as antioxidant and 0.01 wt. percent of a silicone anti-foamant.

The above compositions were tested in a lead corrosion test which was carried out by rapidly rotating a bi-metallic strip consisting of a lead strip and a copper strip bound together in an oil sample maintained at 325° F. while air was bubbled through the sample. The weight loss of the lead strip is then determined and reported in terms of milligram weight loss per sq. inch of lead surface. The compositions tested and the results obtained are summarized in the following table:

Table I

#### LEAD CORROSION TEST

| Test | Composition                                                              | 1 Hr. Lead Corrosion (mg./in. <sup>2</sup> ) |      |     |     |
|------|--------------------------------------------------------------------------|----------------------------------------------|------|-----|-----|
|      |                                                                          | 1                                            | 4    | 8   | 12  |
| 40   |                                                                          |                                              |      |     |     |
| 45   | Diester                                                                  | 3.8                                          | 15.2 | 141 | 326 |
| 2    | Diester +0.275 wt. percent sebacic acid-PEG 200-sebacic acid             | 0.6                                          | 1.2  | 1.3 | 3.1 |
| 3    | Diester +0.5 wt. percent sebacic acid-PEG 200-sebacic acid               | 0                                            | 0.2  | 0.2 | .2  |
| 4    | Diester +0.3 wt. percent sebacic acid-hexanediol-2,5-sebacic acid        | 0.2                                          | 0.4  | 0.8 | 1.0 |
| 5    | Diester +0.44 wt. percent adipic acid-PEG 200-adipic acid                | 0                                            | 0    | 0   | 0   |
| 6    | Diester +0.2 wt. percent adipic acid-hexanediol-2,5-adipic acid          | 0                                            | 0    | 0   | 0.2 |
| 7    | Diester +0.22 wt. percent adipic acid-2-ethyl hexanediol-1,3-adipic acid | 0.2                                          | 0.6  | 1.1 | 1.3 |
| 8    | Complex ester                                                            | 5                                            | 29   | 125 | 251 |
| 9    | Complex ester +1.5 wt. percent adipic acid-PEG 200-adipic acid           | 0                                            | 0.2  | .6  | .8  |
| 55   | Complex ester +1.5 wt. percent sebacic acid-PEG 200-sebacic acid         | 0.2                                          | 1.2  | 2.3 | 3.5 |

The above table demonstrates the remarkable effectiveness of the compositions of the invention in reducing lead corrosion caused by the ester base oils. Thus, the diester base composition (Test 1) showed considerable corrosivity to lead. However, the addition of varying amounts of the acidic partial esters of Examples I through V drastically reduced the amount of corrosion (see Tests 2 to 7). In fact, Test 5 shows that .44 wt. percent of the product of Example III completely eliminated lead corrosion. Tests 8 to 10 demonstrate the effectiveness of the acidic partial esters with a complex ester base oil composition.

Several of the blends of Table I were further tested for corrosiveness to copper, magnesium, iron, aluminum and silver and for changes in viscosity and acidity. These tests were carried out in accordance with MIL-L-7808-C specification procedure, i.e., by immersing weighed strips

of the metal to be tested in a 100 cc. of the sample maintained at 347° F. for 72 hours while bubbling 0.5 liter per hour of air through the sample. The metal strip is then re-weighed to determine the weight change as mg./cm.<sup>2</sup> and the change in viscosity and neutralization number of the composition is determined. The compositions tested and the results obtained are summarized in Table II which follows:

Table II  
OXIDATION-CORROSION STABILITY

| Composition                                           | 347° F. Oxidation-Corrosion Stability |       |      |      |       |              |                              |
|-------------------------------------------------------|---------------------------------------|-------|------|------|-------|--------------|------------------------------|
|                                                       | Corrosion, mg./cm <sup>2</sup>        |       |      |      |       | Neut. Change | Vis./100° F., Percent Change |
|                                                       | Cu                                    | Mg    | Fe   | Al   | Ag    |              |                              |
| Diester                                               | 0.01                                  | 0.01  | 0.01 | 0.00 | 0.01  | 0.8          | 3.4                          |
| Diester +0.275% sebadic acid-PEG-200-sebadic acid     | 0.05                                  | 0.05  | 0.07 | 0.06 | 0.07  | 0.9          | 1.4                          |
| Diester +0.5% sebadic acid-PEG-200-sebadic acid       | 0.13                                  | 0.07  | 0.09 | 0.08 | 0.11  | 0.9          | 2.2                          |
| Complex Ester                                         | -0.34                                 | -0.01 | 0.05 | 0.05 | -0.01 | 1.4          | 10.0                         |
| Complex Ester +1.5% sebadic acid-PEG-200-sebadic acid | 0.04                                  | 0.06  | 0.02 | 0.03 | 0.00  | 0.1          | 15.0                         |

As shown by Table II, there is no significant change in corrosion of the above five metals by use of the acidic partial esters of the invention. The change shown is within the tolerance allowed for products of this sort.

Several of the compositions of Table I and Table II were next tested for load-carrying ability in the Ryder Gear Test in accordance with MIL-7808C specification procedures and in a modified SAE load-carrying test. In the modified SAE test, the Standard SAE lubricant tester was used except that a gear ratio of 3.4:1 was used in place of the conventional ratio of 14.6:1. The test was carried out by running the machine for two minutes under a 50 lb. load and then manually increasing the load 50 lbs. every ten seconds until scuffing occurred. The compositions tested and the results obtained are summarized in Table III which follows:

Table III  
LOAD CARRYING ABILITY

| Composition                                           | SAR-SOD Load, lbs. | Ryder Gear Load, Lbs./in. |
|-------------------------------------------------------|--------------------|---------------------------|
| Diester                                               | 475                | 1,800                     |
| Diester +0.275% sebadic acid-PEG 200-sebadic acid     | 600                | 2,830                     |
| Diester +0.5% sebadic acid-PEG 200-sebadic acid       | 700                | 3,180                     |
| Complex Ester                                         |                    | 3,050                     |
| Complex Ester +1.5% adipic acid-PEG 200-adipic acid   |                    | 3,970                     |
| Complex ester +1.5% sebadic acid-PEG 200-sebadic acid |                    | 3,425                     |

As seen by the above table, the additives of the invention are also useful for imparting load-carrying ability to synthetic ester lubricating oils.

While the prior examples have shown the reaction of 2 molar proportions of a dicarboxylic acid per 1 molar proportion of a glycol, a lesser molar proportion of the dicarboxylic acid may be used. To illustrate, Example I is repeated by reacting 3 moles of the sebadic acid with 2 moles of the Polyethylene Glycol 200.

What is claimed is:

1. A lubricating oil composition comprising a major amount of carboxylic acid ester lubricating oil and within the range of 0.01 to about 2.0 wt. percent, based on the weight of said ester oil, of an acid partial ester dissolved in said oil, and wherein said acid partial ester is the esterification product of about 1.7 to about 2.0 molar propor-

tions of a C<sub>4</sub> to C<sub>12</sub> alkandioic acid with one molar portion of a C<sub>2</sub> to C<sub>36</sub> glycol.

2. A lubricating oil composition according to claim 1, wherein said acid partial ester is formed by the esterification of two molar proportions of said alkandioic acid with one molar proportion of said glycol.

3. A lubricating oil composition according to claim 1, wherein said glycol is a polyalkylene glycol.

4. A lubricating oil composition according to claim 1, wherein said glycol is an alkylene glycol.

5. A lubricating oil composition according to claim 1, wherein said glycol contains 4 to 18 carbon atoms.

6. A lubricating oil composition according to claim 1, wherein said synthetic ester lubricating oil consists of a hydrocarbon chain interrupted by ester linkages.

7. A lubricating oil composition according to claim 1, wherein said ester lubricating oil is a diester having the formula



wherein R is a C<sub>6</sub> to C<sub>13</sub> alkyl group and R' is a C<sub>2</sub> to C<sub>8</sub> saturated hydrocarbon radical.

8. A lubricating oil composition comprising a major amount of a carboxylic acid ester lubricating oil and dissolved therein about 0.01 to about 0.5 wt. percent of the esterification reaction product of about 2 moles of a C<sub>4</sub> to C<sub>12</sub> alkandioic acid with 1 mole of a C<sub>4</sub> to C<sub>18</sub> glycol.

9. A lubricating oil composition according to claim 8, wherein said ester lubricating oil is a diester, said alkandioic acid is an adipic acid and said glycol is a polyethylene glycol having an average molecular weight of about 182.

References Cited in the file of this patent

UNITED STATES PATENTS

- |    |           |                    |               |
|----|-----------|--------------------|---------------|
| 60 | 2,788,326 | Bondi et al. ----- | Apr. 9, 1957  |
|    | 2,918,433 | Buckmann -----     | Dec. 22, 1959 |
|    | 2,929,786 | Young et al. ----- | Mar. 22, 1960 |
|    | 2,960,469 | Young -----        | Nov. 15, 1960 |